

1

3,379,540

**ADDITIVES TO SAND MOULDS AND CORES**  
 Derek Priestley Hellier, Birmingham, England, assignor  
 to Foseco International Limited, Birmingham, England,  
 a British company  
 No Drawing. Filed July 21, 1965, Ser. No. 473,851  
 Claims priority, application Great Britain, Aug. 20, 1964,  
 34,116/64; Nov. 24, 1964, 47,774/64; Dec. 31, 1964,  
 53,040/64

8 Claims. (Cl. 106—38.5)

## ABSTRACT OF THE DISCLOSURE

Finning or veining produced on metal casting cast in sand moulds or around sand cores may be minimised by the incorporation into the sand mould or core of a proportion of colemanite or unexpanded perlite.

This invention relates to said moulds and cores and more particularly to additives for sand moulds and cores which improve the characteristics thereof. The invention may be applied to sand moulds and cores incorporating any organic binder but it is of greatest practical value in connection with oil-bonded sand cores as hereinafter set forth.

The invention is concerned with the production of castings from non-skin-forming metals which are poured at above 750° C. Such metals are the cast irons (grey or modular) and copper based alloys such as lead-, tin- and Phosphor-bronzes.

In producing castings of such metals using moulds or cores of oil-bonded or resin-bonded natural, synthetic or semi-synthetic silica sands (i.e. which contain less than 5% clay), which have a high dry compression strength, a difficulty sometimes arises which is known in the art as "finning" or "veining." When such a sand core is heated by the molten metal it may develop surface cracks. The molten metal tends to enter these cracks and in consequence when the casting is stripped away from the core it may have projections corresponding to these cracks, so called "fins" or "veins" which of course must, where possible, afterwards be removed from the casting by a machining operation. The phenomenon of finning and veining thus leads to an increase in overall production costs. Moreover in some cases, e.g. where the finning or veining occurs in a narrow passage way of the casting, the removal of the fins or veins may not be a practical possibility.

The incidence of finning or veining appears to vary with the nature of the bonding agent. Sand moulds and cores which have inorganic binders, e.g. which are bonded with silicate, appear to show little tendency towards this phenomenon and such moulds and cores are therefore not included within the scope of this invention.

Sand moulds and cores in which the bonding agent is oil, i.e. a drying or semi-drying oil such as linseed, tung or oilcica, or mixtures of any of these, the oil being optionally in association with a cereal carbohydrate or the like, which usually include a metal, e.g. cobalt or lead, naphthenate as hardener, and which require stoving before use, show some tendency to finning and veining. Sand moulds and cores in which the binder is an air-drying oil (as above) together with an accelerator, e.g. an inorganic peroxy compound such as sodium perborate, show a slightly greater tendency to finning and veining. The resin-bonded sand moulds and cores generally exhibit the phenomenon to an appreciably greater extent: e.g. in the case of furane bonding resins which are set by heating the problem is very severe and in the case

2

of furane bonding resins which are cold set the problem, though still severe, is not quite so serious.

It is an object of the present invention to provide oil-bonded or resin-bonded synthetic or washed silica sand moulds and cores of high dry compression strength, especially cores which contain certain additives tending to reduce the incidence of finning or veining to be used for casting non-skin forming metals.

According to the present invention, there is provided an oil-bonded or resin-bonded natural, synthetic or semi-synthetic silica sand mould, or core containing less than 5% of clay, for use in casting non-skin forming metals, having a dry compression strength of more than 14 kg./sq. cm. which includes as an additive to the composition of the sand mould or core, potassium nitrate, colemanite, unexpanded perlite, barium sulphate, sodium metaphosphate or potassium alum, or a mixture of any of said substances.

The reason why these substances function is not understood, especially since they are inherently dissimilar in chemical and physical properties. Potassium nitrate, barium sulphate, sodium metaphosphate and potassium alum are relatively simple chemical substances the characteristics of which are well known. Colemanite is a commercially available mineral of the approximate formula  $2\text{CaO}\cdot 3\text{B}_2\text{O}_3\cdot 5\text{H}_2\text{O}$ . A naturally occurring hydrated calcium tetraborate, which in the anhydrous form melts at nearly 1000° C. and is also known as boro-calcite, and perlite is a mineral which, on heating, exfoliates to reduce its initial density of between 2 and 3 to a value very much below 1. It is believed that each of these substances acts in its own way to facilitate relative movement of the sand grains so that the expansion of the mould or core on heating can be taken up by the material of the mould or core without giving rise to cracking.

Generally speaking the quantity of said substance or mixture of said substances suitable for addition to the material of the mould or core may be within the range 0.5 to 5% of the total weight of the dry mould or core, although a somewhat higher proportion may be required occasionally.

It is to be noted however that a successful additive should not only prevent finning, but also maintain strength, the knock out properties should not be affected, nor must the bonding properties of the oil or the polymerisation of the resin be inhibited. The gas evolution must not be increased and the surface finish should be improved rather than impaired. The additives of this invention tend to fulfill all these requirements.

Where the binder for the sand is a resin it is preferably a furane resin but other resin binders may be employed, e.g. phenol-formaldehyde or urea-formaldehyde resins. If desired there may be used, with any such resin binder, a diluent liquid which will assist in providing a suitably mouldable sand mix. The diluent liquid, if used, should of course not have any deleterious inhibitory effect on the polymerisation or polycondensation of the resin whereby the resin hardens to give a rigid product. Suitable liquids for the purpose are inert mineral oils and the oil product sold commercially under the trademark Dutrex 55.

The use of the special additives of the present invention makes it possible to use a smaller amount of the resin binder while still obtaining a desired strength in the final product. The inclusion of a liquid diluent as just described makes the use of such smaller quantities of resin binder easier to handle in practice.

However, while the additives of the present invention reduce the incidence of finning or veining in such resin-bonded sand moulds and cores the additives are not always wholly successful in totally eliminating the phenomenon. On the other hand, applied to oil-bonded sand

resins and cores as referred to above, substantially complete elimination of the finning and veining is achieved.

The following examples will serve to illustrate the invention:

#### EXAMPLE 1

To Kings Lynn S.S. sand, a fine washed silica sand, bonded with a hot-box furane resin, was added 0.5% by weight of the dry sand of the additives listed below. This mixture was milled until evenly dispersed. 0.15% of a catalyst for a furane-type hot-box resin was then added and the mixture milled again followed by 2 1/4% by weight of a furane-type hot-box resin and the mixture milled again until all the additives were evenly distributed throughout the sand. The mixture was then fed to a conventional foundry core blower for the manufacture of cores, by the hot-box technique. These cores were incorporated in foundry moulds for the manufacture of castings of low phosphorus cast iron which was poured at 1400° C.

The following results show that the three additives of this invention either used singly or in combination all tend to reduce finning on non-skin forming metals.

| Percent composition of additive                            | Dry strength, kg./sq. cm. | Finning      |
|------------------------------------------------------------|---------------------------|--------------|
| No addition.....                                           | 77                        | Very severe. |
| 100% potassium nitrate.....                                | 67                        | Slight.      |
| 100% unexpanded perlite.....                               | 87                        | Nil.         |
| 100% boro-calcite (colemanite).....                        | 115                       | Slight.      |
| 100% boro-clacite (0.25 addition).....                     | 109                       | Moderate.    |
| 50/50% pot. nitrate/unexpanded perlite.....                | 78                        | Slight.      |
| 50/50% pot. nitrate/boro-calcite.....                      | 100                       | Do.          |
| 50/25/25 pot. nitrate/unexpanded perlite/boro-calcite..... | 71                        | Do.          |

#### EXAMPLE 2

The following sand mix was used for the manufacture of cores, for the manufacture of cast iron castings:

|                                                                         |    |       |
|-------------------------------------------------------------------------|----|-------|
| Congleton sand .....                                                    | kg | 181.6 |
| Dextrin .....                                                           | kg | 2.72  |
| Core oil .....                                                          | cc | 1120  |
| Water .....                                                             | cc | 1680  |
| Anti-finning (50/50 mixture of colemanite and unexpanded perlite) ..... | kg | 1.82  |

Cores manufactured from this mixture had a dry compression strength of 57 kg./sq. cm. (this compares with the strength of approximately only 42 kg./sq. cm. when used without the anti-finning additive) and the castings produced were entirely free from veins or fins whereas there had previously been a severe level of scrapped castings because of the incidence of such faults.

I claim as my invention:

1. Oil-bonded and resin-bonded natural, synthetic and semi-synthetic silica sand moulds and cores containing less than 5% of clay, for use in casting non-skin forming metals, having a dry compression strength of more than 14 kg./sq. cm. which include as an additive to the composition thereof, at least 0.5% by weight of a substance selected from the class consisting of colemanite and unexpanded perlite.

2. A mould or core for use in casting non-skin forming metals which comprises essentially silica sand containing less than 5% by weight of clay and bonded by means of a drying oil and a cereal carbohydrate, and having a dry compression strength of more than 14 kg./sq. cm. which includes as an additive to the composition thereof, unexpanded perlite, the said additive being present in a proportion of 0.5 to 5% by weight of the composition.

tion thereof, at least 0.5% by weight of a substance selected from the class consisting of colemanite and unexpanded perlite.

3. A mould or core for use in casting non-skin forming metals which comprises essentially silica sand containing less than 5% by weight of clay and bonded by means of a drying compression strength of more than 14 kg./sq. cm. which includes, as an additive to the composition thereof, at least 0.5% by weight of colemanite.

4. A mould or core for use in casting non-skin forming metals which comprises essentially silica sand containing less than 5% by weight of clay and bonded by means of a drying oil and a cereal carbohydrate, and having a dry compression strength of more than 14 kg./sq. cm. which includes, as an additive to the composition thereof, at least 0.5% by weight of unexpanded perlite.

5. Oil-bonded and resin-bonded natural, synthetic and semi-synthetic silica sand moulds and cores containing less than 5% of clay, for use in casting non-skin forming metals, having a dry compression strength of more than 14 kg./sq. cm. which include as an additive to the composition thereof, a substance selected from the class consisting of colemanite and unexpanded perlite, the said additive being present in a proportion of 0.5 to 5% by weight of the composition.

6. A mould or core for use in casting non-skin forming metals which comprises essentially silica sand containing less than 5% by weight of clay and bonded by means of a drying oil and a cereal carbohydrate, and having a dry compression strength of more than 14 kg./sq. cm. which includes as an additive to the composition thereof, a substance selected from the class consisting of colemanite and unexpanded perlite, the said additive being present in a proportion of 0.5 to 5% by weight of the composition.

7. A mould or core for use in casting non-skin forming metals which comprises essentially silica sand containing less than 5% by weight of clay and bonded by means of a drying oil and a cereal carbohydrate, and having a dry compression strength of more than 14 kg./sq. cm. which includes, as an additive to the composition thereof, colemanite, the said additive being present in a proportion of 0.5 to 5% by weight of the composition.

8. A mould or core for use in casting non-skin forming metals which comprises essentially silica sand containing less than 5% by weight of clay and bonded by means of a drying oil and a cereal carbohydrate, and having a dry compression strength of more than 14 kg./sq. cm. which includes, as an additive to the composition thereof, unexpanded perlite, the said additive being present in a proportion of 0.5 to 5% by weight of the composition.

#### References Cited

| UNITED STATES PATENTS |        |              |            |
|-----------------------|--------|--------------|------------|
| 2,237,592             | 4/1941 | Dunbeck      | 106-38.9   |
| 2,426,000             | 8/1947 | Cutler       | 106-38.7 X |
| 2,789,331             | 4/1957 | Dietert      | 22-193     |
| 2,797,457             | 7/1957 | Kramer       | 22-193     |
| 2,974,050             | 3/1961 | Barlow       | 106-38.5   |
| 3,104,230             | 9/1963 | Dewey et al. | 22-193 X   |

ALEXANDER H. BRODMERKEL, Primary Examiner.

DONALD J. ARNOLD, Examiner.

L. B. HAYES, Assistant Examiner.